

July 12, 1960

O. G. FOLBERTH

2,944,975

METHOD FOR PRODUCING AND RE-MELTING COMPOUNDS HAVING  
HIGH VAPOR PRESSURE AT THE MELTING POINT

Filed Aug. 9, 1956



# United States Patent Office

2,944,975

Patented July 12, 1960

NOTICE: Patent rights do not to his assignee and successors

1

2,944,975

## METHOD FOR PRODUCING AND REMELTING COMPOUNDS HAVING HIGH VAPOR PRESSURE AT THE MELTING POINT

Otto Gert Folberth, Erlangen, Germany, assignor to Siemens-Schuckertwerke Aktiengesellschaft, Berlin-Siemensstadt and Erlangen, Germany, a corporation of Germany

Filed Aug. 9, 1956, Ser. No. 603,073

Claims priority, application Germany Sept. 14, 1955.

19 Claims. (Cl. 252—62.3)

This invention relates to the production or remelting of multi-component substances, including alloys and stoichiometric compounds. It particularly concerns the homogenizing and purifying of such substances.

Before proceeding with a description of the new processes for homogenizing and purifying, it is desirable to describe the field and scope of the processes. The field is set forth in my copending U.S. application Serial No. 554,361, filed December 20, 1955, Patent No. 2,858,275, of which the instant application is a continuation-in-part.

My invention relates generally to semiconductor devices. Such devices have a crystalline body of electrical-ally semiconducting substance subjected to electric or magnetic fields, to corpuscular or wave radiation or to a plurality of such phenomena, for performing electrical, photo-electrical, optical or other physical effects. Examples of semiconductive devices, within the scope of my invention, are transistors, junction rectifiers, thermistors, detectors, photo-electric cells, thermo-electric junctions, photo-modulators, crystalline optical filters and other optical components.

In the past, semiconductor devices have predominantly been provided with a crystalline body of germanium (Ge) or silicon (Si) appertaining to the same subgroup in the fourth group of the periodic system as the semiconducting elements diamond (C) and gray tin (Sn).

It has also become known, and is disclosed in the copending application of H. Welker, Serial No. 275,785, filed March 10, 1952 (assigned to the assignee of the present invention), which has issued as Patent No. 2,798,989, on July 9, 1957, that certain binary compounds of elements from the third group (B, Al, Ga, In) with elements from the fifth group (N, P, As, Sb) are also applicable as semiconductors. These sixteen compounds, now usually called "A<sup>III</sup>B<sup>V</sup>" or simply "III-V" semiconductors, can be looked upon as being approximate replicas of the semiconducting fourth-group elements C, Si, Ge, Sn with respect to width of the forbidden zone and lattice spacing.

When considering the physical properties, particularly those relating to semiconductance, of the individual fourth-group elements in their atom-number sequence: C, Si, Ge, Sn, it appears that relative to any one particular property, such as forbidden-zone width, lattice spacing or melting point, this property differs from element to element in the same sense of progression. Now, the semiconductor III-V compounds add to the previously available discrete properties of the four elementary semiconductors a variety of intermediate property values thus affording a greater choice. It must be considered, however, that certain physical properties, such as width of the forbidden zone and carrier mobility, vary in mutually inverse relation from fourth-group element to element and also from III-V compound to compound. For instance, in the sequence from diamond (C) to gray tin (Sn), the width of the forbidden zone decreases, which

is tantamount to decrease in melting point and decrease in temperature-stability of the electric properties, whereas, in the same sequence, the carrier mobility increases. The III-V semiconductors behave analogously. Hence, a III-V semiconductor of relatively great electron mobility also has a relatively great temperature dependence of its electric conductance properties. Thus, according to recent measurements, an optimum electron mobility of about 65,000 cm.<sup>2</sup>/volt second is obtainable with indium antimonide (InSb) but is accompanied by a relatively great temperature dependence. For applications requiring least possible sensitivity to changes in temperature, it is preferable to use compounds of a wide forbidden zone, that is compounds corresponding in this respect to Ge or even to Si. Thus, with indium arsenide (InAs), having a forbidden-zone of 0.45 e.v. as compared with 0.27 e.v. of InSb, a much lesser temperature dependence than that of InSb is obtained, but the carrier mobility is considerably lower, namely approximately

10 30,000 cm.<sup>2</sup>/volt second. If one selects a III-V compound still more closely related to Ge as to forbidden zone, then the temperature dependence is further reduced but the carrier mobility is also much lower. For instance, gallium antimonide (GaSb) has a forbidden zone of about 0.7 e.v. width corresponding substantially to that of Ge, but the electron mobility is only about 3,000 cm.<sup>2</sup>/volt sec.

For many applications of semiconductors, therefore, it would be desirable to have available a semiconductor substance which combines high carrier mobility, such as a mobility similar to that of InAs, in conjunction with a relatively low temperature dependence. It is among the objects of my invention to provide such semiconductor substances.

35 Another object of my invention is to afford obtaining not only the discrete property values peculiar to the individual elemental and compound semiconductor substances heretofore available, but also any other property value within a wide and substantially continuous range, so that it becomes possible to "tailor" the crystalline semiconductor body, as regards its properties, to the optimum requirements of any particular application intended.

40 To achieve these results, and in accordance with a feature of my invention, I form the crystalline body of the semiconductor device by crystallizing it from a mixture of III-V semiconductor compounds of different solid solubility relative to each other. That is, each compound of the mixture consists of a different pair of 45 the above-specified eight elements from the third and fifth periodic-system groups respectively, and the resulting solid body consists of a mixed crystal.

According to another feature of my invention, the mixed-crystal semiconductor body is preferably formed 50 of two different III-V compounds which have one of their component elements in common. Such mixed crystals may have a composition of the type (A<sub>x</sub>B<sub>1-x</sub>)<sup>III</sup>C<sub>1</sub>V where A and B are different respective elements from the third group and C is an element from the fifth group of the periodic system, and the subscripts denote atom proportions, the value x being larger than zero and smaller than unity. Mixed-crystal formations of this 55 type are, for example, the compositions (In<sub>x</sub>Ga<sub>1-x</sub>)Sb formed of InSb and GaSb, or compositions

60 (In<sub>x</sub>Ga<sub>1-x</sub>)As<sub>1</sub> formed of InAs and GaAs, or compositions (In<sub>x</sub>Ga<sub>1-x</sub>)P<sub>1</sub> formed of InP and GaP.

65 However, according to another feature of my invention, I compose the semiconducting mixed crystal so that the two component III-V compounds have an element of

the third group in common. This mixed crystal is of the type  $A_1^{III}(C_yD_{1-y})^V$  wherein A is an element of the third group, C and D are different respective elements of the fifth group, and the subscripts denote atom proportions, the value of y being larger than zero and smaller than unity. Mixed crystals of this type form themselves readily from a melt of the components and can readily be processed and used in practice in much the same manner as the III-V compounds themselves.

It is known that two elements "U" and "V" which are isomorphous as well as soluble in each other in the solid state, may form mixed crystals within a continuous range of composition. This has been observed for such alloys as Ag—Au, Sb—Bi and Ge—Si. Within that range of composition, the respective properties of such mixed crystals show a continuous change, depending upon the particular proportions of the composition, from the properties of the pure element "U" to the properties of the pure element "V." This has also been observed, relative to forbidden zone and carrier mobility, with mixed crystals of the type  $Ge_xSi_{(1-x)}$  formed by the semiconducting elements Ge and Si. However, the existence of mixed crystals of semiconducting III-V compounds was not known, and the utility and advantage of such compound mixed-crystals for use in electrical, photo-electrical, optical and the like semiconductor devices was likewise unknown.

I further discovered that the III-V compound mixed crystals can be produced from a melt and can be processed substantially in the same manner as the elemental semiconductors or the individual III-V semiconductor compounds themselves. That is, the compound mixed crystals can be purified, homogenized by tempering, or can be processed toward monocrystalline structure, for instance by zone melting, melting and normal freezing (oriented solidification), or pulling a monocrystal out of the melt. For instance, a monocrystal can be produced in the known manner by placing a monocrystalline germ or seed in contact with the melt of the compound mixture and then pulling the seed away from the melt at the speed of crystallization so that a monocrystal of the desired mixed type will grow on the seed. I found that the melting, zone-melting or other heat treatment does not result in decomposition or segregation of the mixed crystal, and also that the mixed crystals can be doped with substantial impurities (lattice-defect atoms), for instance as needed for producing p-n junctions. Doping the crystal with an element of the second periodic group, preferably cadmium or zinc (acceptors), produces p-type conductance. Elements of the sixth group, preferably sulphur, selenium or tellurium, act as donors, i.e. produce n-type conductance.

I have found that among the compound mixed crystal semiconductors according to the invention those of the types  $In_1(As_yP_{1-y})$  and  $Ga_1(As_yP_{1-y})$  are particularly advantageous. Mixed crystals of such compositions can readily be produced by melting in each case the two component compounds together or by producing a melt from a mixture of three elements in the proper atomic proportion. The mixed crystals can further be readily subjected to any of the above-mentioned processing methods. In comparison with the semiconductor compounds InAs and GaAs as such, the width of the forbidden zone and hence the temperature dependence of the electric properties can be considerably modified by the selection of the amount of phosphorus. Consequently, for any particular application of the semiconductor device the most desirable intermediate values of the semiconductor properties can thus be obtained and the composition can be tailored as to its properties to definite predetermined values.

This application is an improvement of or modification of the invention described in the pending U.S. application Serial No. 534,852, filed on September 16, 1955, in

which the instant applicant is joined with another. I incorporate by reference all of the subject matter found in Serial No. 534,852 into the instant application. That application relates to a method for producing an alloy or compound in crystalline form by melting the components together within a sealed system, the compound or alloy being such that in condition of equilibrium the partial vapor pressure of one, or more, components above the melt is considerably higher than the partial vapor pressure of the other component, or components, and is also considerably higher than the partial vapor pressure of a gaseous compound formed of these components.

The method according to the said copending application Serial No. 534,852 represents an improvement over 15 the Faraday method and differs therefrom by the fact that the weighed-in quantities of the components as well as the temperature program are so chosen that, on the one hand, the melt can take the desired proportion of the low-volatile component out of the vapor phase and that, on 20 the other hand, the remainder of this component, or components, is just sufficient to form the share of this component, or components, of the equilibrium vapor phase above the melt so that there is no residual or bottom body of the low boiling or more volatile component, or components, on the bottom of the processing vessel at the 25 termination of the melting operation. As a result, and in contrast to the Faraday method, it is not necessary to maintain the temperature of the coldest spot of the melting vessel at an accurate value; and the processing becomes 30 independent of the complicated vapor-pressure conditions obtaining with polymorphous conversions of the bottom body. Said copending application Serial No. 534,852 also describes the application of this process to zone melting.

35 The present invention has for its further object to provide a method which is suitable for homogenizing and purifying of compounds and alloys composed of more than two components, particularly components having a wide range of existing concentrations. Among such compounds are, above all, the mixed crystals formed by  $A_1^{III}B_1^{V}$  compounds as described in my copending application Serial No. 554,361, filed December 20, 1955, and assigned to the assignee of the present invention. The term "wide range of existing concentrations of a compound or alloy, particularly a mixed crystal," means that the range of existence relative to at least two of the components is wide with respect to the relative concentrations or proportions which these respective components may assume in the mixed crystal.

40 The present invention will be specifically described in reference to the mixed crystal,  $In(As_{0.8}P_{0.2})$ . However, the invention has wider scope and implication, since it includes all of the manifold examples, species and classes described in my copending application Serial No. 554,361.

45 For example, this further includes elements from group six, such as sulfur, selenium, and tellurium as the more volatile component.

50 For producing a mixed crystal of the composition  $In(As_{0.8}P_{0.2})$  the apparatus illustrated on the drawing 55 may be employed, this device being identical with the one described in U.S. application Serial No. 534,852. Accurately weighed quantities of 15,000 grams indium (In), 7,893 g. arsenic (As) and 0.870 g. phosphorus (P) are sealed into an ampule 1 of quartz of 60 cm.<sup>3</sup> volume.

55 The indium is placed in a carburized boat 2 of quartz. The weighed amount of arsenic and phosphorus may be located on any other free spot on the bottom of the quartz ampule. The sealed and fused-off quartz ampule is placed in a two-temperature furnace which is equipped 60 with a high-frequency induction heater 4 located in the center range of the ampule for heating the indium-containing boat, and two resistance heaters 5-6 so located as to maintain the end portions of the ampule at an elevated temperature. The melting is carried out 65 as described in U.S. application Serial No. 554,361,

Patent No. 2,858,275. The boat is heated by the high-frequency induction coil 4 to a temperature of about 960° C., and the other parts of the ampule are kept at about 700° C. by means of the heaters 5, 6. As a result a melt is produced in the boat which has the composition  $\text{In}(\text{As}_{0.8}\text{P}_{0.2})$ , and there is also formed the corresponding vapor phase without any bottom body remaining of the weighed-in low-volatile components As and P. If this melt were permitted to solidify slowly, progressing from one end, as in normal freezing, then a crystal would be formed, whose first solidified end contains more phosphorus, of the approximate composition  $\text{In}(\text{As}_{0.7}\text{P}_{0.3})$ , and whose last solidified end contains more arsenic, for example of the approximate composition  $\text{In}(\text{As}_{0.9}\text{P}_{0.1})$ . Such crystals are no doubt desirable for some applications. Generally, however, it is preferred to obtain homogeneous crystals from the melt. According to the present invention this is achieved as follows:

The melt produced as described above, is first caused to rapidly solidify in an unoriented manner, the speed of solidification being so great that, although the crystalline lattice structure is greatly heterogeneous from the fine-structural viewpoint, the structure is quasi-homogeneous from the macroscopic or coarse-structural viewpoint. Now, in order to also obtain a homogeneous fine-structure, a further processing step is employed according to which the solidified crystal is subjected to zone-melting in a narrow melting zone, preferably in two successive and mutually opposed directions, the melting zone having a width of at most about one-fifth of the total axial length of the semiconductor body but being preferably much narrower. For example, the solidified crystal is first heated to the melting point at the left end, the heating being confined to a narrow zone or portion of the length of the crystal and being progressively advanced along the crystal to the right end (see W. A. Pfann, Journal Metals, July 1952, page 747). Then this process is repeated, but this time starting at the right end and traveling back to the left end. In this manner there is produced a homogeneous mixed crystal, which is in the present case of the composition  $\text{In}(\text{As}_{0.8}\text{P}_{0.2})$ , with the exception of a very small remainder which approximately corresponds to the width of the melting zone last solidified.

A mixed crystal produced and homogenized in the above-described manner can be further purified by additional zone-melting. During such additional zone-melting, in similarity to the above-described normal freezing, the mixed crystal again becomes heterogeneous. At the first solidified end of the crystal, more phosphorus is built into the crystal lattice structure, whereas at the last solidified end more arsenic will occur than corresponds to the original composition of the crystal. During the next following zone-melting step, therefore, the first melted narrow zone has an As/P ratio which no longer corresponds to that of the vaporous phase above the melt since this vaporous phase was in equilibrium with the last solidified zone. Since, on the other hand, the total vapor pressure also increases with increasing P content of the melt, the first re-melted zone during the second zone-melting step gives off to the vapor phase more P than it takes As from the vapor phase. Consequently the melt now contains more In than corresponds to the original composition. This has the consequence that indium inclusions occur in the crystal at the beginning of the second zone-melting step. When the zone-melting progresses to the other end of the crystal, the conditions become reversed: the melt takes up more P and As from the vaporous phase than corresponds to the original composition, with the effect that during solidification there will occur vapor inclusions within the crystals. Therefore, a mixed crystal which has been zone-melted a number of times in the above-described manner, exhibits indium inclusions at one end and is porous at the other end. Only the middle portion of the crystal possesses the desired homogeneous composition and consistence.

In certain cases the above-described purifying method is not satisfactory. For one thing, only part of the original crystal can be used. Furthermore, the purifying effect of the zone-melting is not fully utilized because this effect is a maximum in one of the crystal ends which in the present case is of no use. In such cases, and in accordance with another feature of the invention, the following method may be applied:

In order to produce a mixed crystal according to the foregoing example, that is generally of the type



the two binary compounds InAs and InP are individually produced according to the Welker Patent 2,798,989 referred to above, and are purified by zone melting. Then the mixed crystal is produced from these two compounds heating in an ampule in the manner described in U.S. application Serial No. 554,361 and is homogenized as described above. It is inessential that in this case, when weighing the amounts of the components, the three components are present in the form of chemical compounds. The same method is applicable with all compounds or alloys having more than two components.

Like the method described in Welker Patent 2,798,989, the present invention can be applied for the production of mono-crystals with or without crystal germ. By the addition of proper quantities of foreign substances, any desired doping of the crystals to be produced or re-melted can be obtained.

It has been stated above, that the method according to the invention is generally applicable for homogenizing and purifying mixed crystals of  $\text{A}^{\text{III}}\text{B}^{\text{V}}$  compounds. Aside from the above-mentioned example  $\text{In}(\text{As}_{0.8}\text{P}_{0.2})$ , the method is particularly favorable for mixed crystals of the type  $\text{Ga}_1(\text{As}_y\text{P}_{1-y})$  and  $\text{Al}_1(\text{As}_y\text{P}_{1-y})$  in which  $0 < y < 1$ . Furthermore the method is generally applicable to multi-component systems, that is systems with four and more components having a wide range of existing concentrations, provided the components satisfy the above-mentioned requirements as to volatility.

I claim:

1. A method for processing a substance of the group consisting of compounds and alloys of more than two components in crystalline form comprising melting the components together within a sealed system, the partial vapor pressure of at least one component above the melt in the state of equilibrium being considerably higher than the partial vapor pressure of the other component and considerably higher than the partial pressure of a gaseous compound of these components, there being no bottom body of any of the low-boiling, more volatile components present at the termination of the melting operation, the melt being thereafter made to solidify rapidly and in an unoriented manner, the speed of solidification being sufficient to obtain a structure which is quasi-homogeneous macroscopically but with a crystalline lattice structure heterogeneous from the fine-structural viewpoint, and being subsequently zone melted in a narrow melting zone, the melting zone having a width of at most about one-fifth the axial length of the substance.
2. A method according to claim 1 in which the zone melting in a narrow melting zone is carried out successively in two mutually opposed directions to homogenize the product.
3. A method according to claim 2, the homogenized product being thereafter purified by additional zone melting.
4. A method according to claim 1 in which the components of the substance to be processed are binary.
5. A method according to claim 1 applied to alloys comprising mixed crystals.
6. A method for producing a mixed crystal semiconductor body taken from the group consisting of those of the formula  $(\text{A}_x\text{B}_{1-x})^{\text{III}}\text{C}_1^{\text{V}}$  and those of the formula  $\text{A}^{\text{III}}(\text{C}_y\text{D}_{1-y})^{\text{V}}$ , where A and B are component elements

of the third group, and C and D are component elements of the fifth group of the periodic system and  $x$  and  $y$  are each greater than zero and less than one, by melting component substances forming said body within a sealed system, the partial vapor pressure of at least one component element above the melt in the state of equilibrium being considerably higher than the partial vapor pressure of another component element and considerably higher than the partial pressure of a gaseous compound of these component elements, there being no bottom body of any of the low-boiling, more volatile component elements present at the termination of the melting operation, the melt being thereafter made to solidify rapidly and in an unoriented manner in the sealed system, the speed of solidification being sufficient to obtain a body having a structure which is quasi-homogeneous macroscopically but with a crystalline lattice structure heterogeneous from the fine-structural viewpoint, and subsequently zone melting said body in a narrow melting zone in a sealed system successively in two mutually opposed directions to homogenize the product.

7. The process of claim 1, the said substance being a semiconductor compound.

8. The process of claim 1, the said substance having a mixed crystal of a plurality of semiconductor compounds.

9. A method for producing a mixed crystal semiconductor body of the formula  $\text{In}_1(\text{As}_y\text{P}_{1-y})$ , in which  $y$  is greater than zero and less than one, by melting component substances forming said body within a sealed system, the partial vapor pressure of at least one component element above the melt in the state of equilibrium being considerably higher than the partial vapor pressure of another component element and considerably higher than the partial pressure of a gaseous compound of these component elements, there being no bottom body of any of the low-boiling, more volatile component elements present at the termination of the melting operation, the melt being thereafter made to solidify rapidly and in an unoriented manner in the sealed system, the speed of solidification being sufficient to obtain a body having a structure which is quasi-homogeneous macroscopically but with a crystalline lattice structure heterogeneous from the fine-structural viewpoint, and subsequently zone melting said body in a narrow melting zone in a sealed system successively in two mutually opposed directions to homogenize the product.

10. A method for producing a mixed crystal semiconductor body of the formula  $\text{Ga}_1(\text{As}_y\text{P}_{1-y})$ , in which  $y$  is greater than zero and less than one, by melting component substances forming said body within a sealed system, the partial vapor pressure of at least one component element above the melt in the state of equilibrium being considerably higher than the partial vapor pressure of another component element and considerably higher than the partial pressure of a gaseous compound of these component elements, there being no bottom body of any of the low-boiling, more volatile component elements present at the termination of the melting operation, the melt being thereafter made to solidify rapidly and in an unoriented manner in the sealed system, the speed of solidification being sufficient to obtain a body having a structure which is quasi-homogeneous macroscopically but with a crystalline lattice structure heterogeneous from the fine structural view-point, and subsequently zone melting said body in a narrow melting zone in a sealed system successively in two mutually opposed directions to homogenize the product.

11. A method for producing a mixed crystal semiconductor body of the formula  $Al_1(As_yP_{1-y})$ , in which  $y$  is greater than zero and less than one, by melting component substances forming said body within a sealed system, the partial vapor pressure of at least one component element above the melt in the state of equilibrium

being considerably higher than the partial vapor pressure of another component element and considerably higher than the partial pressure of a gaseous compound of these component elements, there being no bottom body

5 of any of low-boiling, more volatile component elements present at the termination of the melting operation, the melt being thereafter made to solidify rapidly and in an unoriented manner in the sealed system, the speed of solidification being sufficient to obtain a body having a  
10 structure which is quasi-homogeneous macroscopically but with a crystalline lattice structure heterogeneous from the fine-structural viewpoint, and subsequently zone melting said body in a narrow melting zone in a sealed system successively in two mutually opposed directions  
15 to homogenize the product.

#### 12. A method for producing a mixed crystal semi-

12. A method for producing a mixed crystal semiconductor body of the formula  $(In_xGa_{1-x})Sb_1$ , in which  $x$  is greater than zero and less than one, by melting component substances forming said body within a sealed system, the partial vapor pressure of at least one component element above the melt in the state of equilibrium

25 component element above the melt in the state of equilibrium being considerably higher than the partial vapor pressure of another component element and considerably higher than the partial pressure of a gaseous compound of these component elements, there being no bottom body of any of the low-boiling, more volatile component elements

present at the termination of the melting operation, the melt being thereafter made to solidify rapidly and in an unoriented manner in the sealed system, the speed of solidification being sufficient to obtain a body having a structure which is quasi-homogeneous macroscopically

35 but with a crystalline lattice structure heterogeneous from the fine-structural viewpoint, and subsequently zone melting said body in a narrow melting zone in a sealed system successively in two mutually opposed directions to homogenize the product.

13. A method for producing a mixed crystal semi-

40 conductor body of the formula  $(In_xGa_{1-x})As_1$ , in which  $x$  is greater than zero and less than one, by melting component substances forming said body within a sealed system, the partial vapor pressure of at least one component element above the melt in the state of equilibrium being

considerably higher than the partial vapor pressure of another component element and considerably higher than the partial pressure of a gaseous compound of these component elements, there being no bottom body of any of the low-boiling, more volatile component elements present.

ent at the termination of the melting operation, the melt being thereafter made to solidify rapidly and in an un-oriented manner in the sealed system, the speed of solidification being sufficient to obtain a body having a structure which is quasi-homogeneous macroscopically but with a crystalline lattice structure between the

with a crystalline lattice structure heterogeneous from the fine-structure viewpoint, and subsequently zone melting said body in a narrow melting zone in a sealed system successively in two mutually opposed directions to homogenize the product.

homogenize the product.

14. A method for producing a body comprising a semiconductor compound by melting component substances forming said body within a sealed system, the partial vapor pressure of at least one component element above the melt in the state of equilibrium being

ment above the liquid in the state of equilibrium being considerably higher than the partial vapor pressure of another component element and considerably higher than 65 the partial pressure of a gaseous compound of these component elements, there being no bottom body of any of the low-boiling, more volatile component elements

70 of the low-boiling, more volatile component elements present at the termination of the melting operation, the melt being thereafter made to solidify rapidly and in an unoriented manner in the sealed system, the speed of solidification being sufficient to obtain a body having a structure which is quasi-homogeneous macroscopically

structure which is quasi-homogeneous macroscopically but with a crystalline lattice structure heterogeneous from the fine-structural viewpoint, and subsequently zone melting said body in a narrow melting zone in a sealed

system successively in two mutually opposed directions to homogenize the product.

15. A method for producing a body comprising a mixed crystal of a plurality of semiconductor compounds by melting component substances forming said body within a sealed system, the partial vapor pressure of at least one component element above the melt in the state of equilibrium being considerably higher than the partial vapor pressure of another component element and considerably higher than the partial pressure of a gaseous compound of these component elements, there being no bottom body of any of the low-boiling, more volatile component elements present at the termination of the melting operation, the melt being thereafter made to solidify rapidly and in an unoriented manner in the sealed system, the speed of solidification being sufficient to obtain a body having a structure which is quasi-homogeneous macroscopically but with a crystalline lattice structure heterogeneous from the fine-structural viewpoint, and subsequently zone melting said body in a narrow melting zone in said sealed system successively in two mutually opposed directions to homogenize the product.

16. A method for processing a substance of the group consisting of compounds and alloys of more than two components in crystalline form comprising melting the components together within a sealed system, the partial vapor pressure of at least one component above the melt in the state of equilibrium being considerably higher than the partial vapor pressure of the other component and considerably higher than the partial pressure of a gaseous compound of these components, there being no bottom body of any of the low-boiling, more volatile components present at the termination of the melting operation, the melt being thereafter made to solidify rapidly and in an unoriented manner, the speed of solidification being sufficient to obtain a structure which is quasi-homogeneous macroscopically but with a crystalline lattice structure heterogeneous from the fine-structural viewpoint, and being subsequently zone melted in a narrow melting zone, the melting zone having a width of at most about one-fifth the axial length of the substance, said substance being composed of at least one component taken from the group consisting of boron, aluminum, gallium, indium, and at least one component from the group consisting of nitrogen, phosphorus, arsenic, and antimony, and all of the components being taken from the said two groups.

17. A process for producing a mixed crystal of the composition  $In_1(As_yP_{1-y})$ , in which  $0 < y < 1$ , the method being carried out in a melting and vaporizing space that is sufficiently enclosed to prevent egress of the vapor evolved in the process, comprising melting indium in a zone of said space, vaporizing arsenic and phosphorus in

said space but separately from said melting of the indium, the proportions of the indium, arsenic and phosphorus being so chosen that there is no residual solid body of the arsenic and phosphorus at the termination of the melting operation, then causing the melt to rapidly solidify in the said space in an unoriented manner, the speed of solidification being sufficient to obtain a structure which is quasi-homogeneous macroscopically but with a crystalline lattice structure heterogeneous from the fine-structural viewpoint, and thereafter zone melting in a narrow melting zone in two successive and mutually opposed directions.

18. A process for producing a mixed crystal of the composition  $Ge_1(As_yP_{1-y})$ , in which  $0 < y < 1$ , the method being carried out in a melting and vaporizing space that is sufficiently enclosed to prevent egress of the vapor evolved in the process, comprising melting gallium in a zone of said space, vaporizing arsenic and phosphorus in said space but separately from said melting of the gallium, the proportions of the gallium, arsenic, and phosphorus being so chosen that there is no residual solid body of the arsenic and phosphorus at the termination of the melting operation, then causing the melt to rapidly solidify in the said space in an unoriented manner, the speed of solidification being sufficient to obtain a structure which is quasi-homogeneous macroscopically but with a crystalline lattice structure heterogeneous from the fine-structural viewpoint, and thereafter zone melting in a narrow melting zone in two successive and mutually opposed directions.

19. A process for producing a mixed crystal of the composition  $Al_1(As_yP_{1-y})$ , in which  $0 < y < 1$ , the method being carried out in a melting and vaporizing space that is sufficiently enclosed to prevent egress of the vapor evolved in the process, comprising melting aluminum in a zone of said space, vaporizing arsenic and phosphorus in said space but separately from said melting of the aluminum, the proportions being so chosen that there is no residual solid body of the arsenic and phosphorus at the termination of the melting operation, then causing the melt to rapidly solidify in the said space in an unoriented manner, and thereafter zone melting in a narrow melting zone in two successive and mutually opposed directions.

#### References Cited in the file of this patent

#### UNITED STATES PATENTS

|           |            |               |
|-----------|------------|---------------|
| 2,710,253 | Willardson | June 7, 1955  |
| 2,739,088 | Pfann      | Mar. 20, 1956 |
| 2,776,206 | Klingbeil  | Jan. 1, 1957  |
| 2,798,989 | Welker     | July 9, 1957  |
| 2,817,608 | Pankove    | Dec. 24, 1957 |

#### FOREIGN PATENTS

|         |               |             |
|---------|---------------|-------------|
| 111,288 | Great Britain | May 9, 1918 |
|---------|---------------|-------------|